

A. MEYER.

PROCESS FOR MANUFACTURE OF PANELS MADE OF ENAMELED OR VITRIFIED SHEET METAL DESIGNED  
TO BE USED AS COVERING MEANS FOR RAILWAYS, CARRIAGES, TRAMWAYS, AUTOMOBILES,  
AND THE LIKE.

APPLICATION FILED JAN. 29, 1913.

1,221,562.

Patented Apr. 3, 1917.

Fig. 1



Fig. 2



Witnesses:

S. C. McBride

G. C. Denny

Inventor:

Alexandre Meyer

By Foster Freeman Watson & Clark  
Attest

# UNITED STATES PATENT OFFICE.

ALEXANDRE MEYER, OF PARIS, FRANCE.

PROCESS FOR MANUFACTURE OF PANELS MADE OF ENAMELED OR VITRIFIED SHEET METAL DESIGNED TO BE USED AS COVERING MEANS FOR RAILWAYS, CARRIAGES, TRAMWAYS, AUTOMOBILES, AND THE LIKE.

1,221,562.

Specification of Letters Patent.

Patented Apr. 3, 1917.

Application filed January 29, 1913. Serial No. 745,047.

To all whom it may concern:

Be it known that I, ALEXANDRE MEYER, engineer, citizen of the French Republic, residing at 10 Rue Thimonnier, Paris, Department of the Seine, France, have invented certain new and useful improvements in processes for manufacture of panels made of enameled or vitrified sheet metal designed to be used as covering means for railways, carriages, tramways, automobiles, and the like, of which the following is a specification.

This invention relates to improvements in the manufacture of enameled metal plates of the nature or for the purpose, for example, of those described in an earlier application, Serial Number 676,092.

It has been discovered that one of the chief causes of destruction of enameled plates, particularly when exposed to changes of atmospheric temperature and vibration, is due to a lack of molecular equilibrium between the plate and enamel coating. To overcome this defect and employ an enamel coating solution like that described in the aforesaid application is the object of the present invention.

In the accompanying drawing:

Figure 1 is a sectional view, on an enlarged scale, of a portion of an enameled metal plate produced in accordance with the invention;

Fig. 2 is a similar view illustrating a slight modification.

In both figures of the drawing 1 designates the metal plate, one surface of which is provided with a coating or layer 2 of anti-oxid, or oxid resisting, material of the nature of that described in said prior application, the formula of which is approximately as below having the nearest coefficient of expansion to the sheet steel known as Martins:

|    |                        |      |       |
|----|------------------------|------|-------|
| 45 | Borax                  | 45   | parts |
|    | Quartz                 | 25   | "     |
|    | Torrified flint        | 5    | "     |
|    | Feldspar               | 16   | "     |
|    | Carbonate of potassium | 5    | "     |
| 50 | Saltpeper              | 2.75 | "     |
|    | Oxid of cobalt         | 0.25 | "     |
|    | Bi-oxid of manganese   | 0.75 | "     |
|    | Oxid of iron           | 0.25 | "     |

On this coating 2 are superposed a plu-

rality of layers 4, 5, 6, of enamel, the solutions or mixtures from which the said layers are produced being so constituted that the complete coating comprises alternately arranged relatively hard and relatively soft, or more readily fusible, layers.

For example, the layer 4 may be such as will be relatively hard or but slightly fusible having the formula of that described in the aforesaid application, namely,

|                                                                                        |       |    |
|----------------------------------------------------------------------------------------|-------|----|
| Silicic acid                                                                           | 2.00  | 65 |
| Silicate of alumina                                                                    | 1.00  |    |
| Saline oxid of lead                                                                    | 0.25  |    |
| Suitable alkali (hydrated borate of sodium, potassium carbonate, or potassium nitrate) | 0.15  | 70 |
| Rutile                                                                                 | 0.015 |    |

and the layer 5 will be of relatively soft enamel or have its constituents so proportioned that it has a relatively low melting point. This relatively soft layer may be produced in accordance with the following formula, namely,

|                                                                                        |      |    |
|----------------------------------------------------------------------------------------|------|----|
| Silicic acid                                                                           | 0.30 | 80 |
| Silicate of alumina                                                                    | 2.00 |    |
| Saline oxid of lead                                                                    | 0.25 |    |
| Suitable alkali (hydrated borate of sodium, potassium carbonate, or potassium nitrate) | 2.50 | 85 |
| Rutile                                                                                 | 0.02 |    |

If, as illustrated in Fig. 2, an additional layer 6 is employed this will be similar to the layer 4, that is, relatively hard or having a high melting point. If desired, as illustrated in Fig. 1, a metal reinforcement 3 may be embedded in one of the enamel layers. In preparing the plate according to the method outlined in Fig. 1, the wire trellis 3 would be placed upon the plate after the anti-oxid layer 2 had been applied thereto and then the solution for forming the enamel layer 4 poured thereon, such solution passing through all of the interstices in the strengthening device so that the latter is thoroughly embedded therein.

It will be understood that the degree of hardness of the enamel layers will depend upon the proportion of alkali employed in the mixture or solution and as above pointed out the layer can be rendered relatively hard or relatively soft as desired by properly proportioning this element.

Having thus described the invention what is claimed is:—

1. The herein described method of preparing enameled metal plates in which a perfect molecular equilibrium exists between the metal plate and enamel coating comprising applying to the plate more than two superimposed layers of enamel, the alternate layers being respectively fusible at a relatively high and relatively low temperature.
2. As an article of manufacture, a metal plate coated on one face with enamel, said coating being in molecular equilibrium with the metal of the plate and being formed by an anti-oxid layer applied directly to the metal and more than two superposed layers of enamel, the alternate layers being respectively fusible at a relatively high and relatively low temperature.
3. A metal sheet or plate having a surface

provided with an enamel coating comprising a surface provided with an enamel coating comprising a plurality of layers, the primary one having a coefficient of expansion substantially the same as that of the metal sheet, and the superimposed layers being fusible at different temperatures and alternately arranged.

4. A metal sheet or plate having a surface provided with an enamel coating comprising a plurality of layers, alternately fusible at relatively high and relatively low temperatures, and a metal reinforcing means embedded in said coating.

In testimony whereof I affix my signature in presence of two witnesses.

ALEXANDRE MEYER.

Witnesses:

BASIL CHOMIEZ,  
LUCIUS MENNINGER.